



US006746491B2

(12) **United States Patent**  
Lack

(10) **Patent No.:** US 6,746,491 B2  
(45) **Date of Patent:** \*Jun. 8, 2004

(54) **BATH FOR PRODUCING WRINKLE  
FREE-WATER RESISTANT FABRICS AND  
GARMENTS**

(75) Inventor: **Ronnie Franklin Lack**, Mize, MS (US)

(73) Assignee: **Warmkraft, Inc.**, Taylorsville, MS  
(US)

(\*) Notice: Subject to any disclaimer, the term of this  
patent is extended or adjusted under 35  
U.S.C. 154(b) by 0 days.

This patent is subject to a terminal dis-  
claimer.

(21) Appl. No.: **10/102,375**

(22) Filed: **Mar. 20, 2002**

(65) **Prior Publication Data**

US 2002/0102892 A1 Aug. 1, 2002

**Related U.S. Application Data**

(62) Division of application No. 09/388,738, filed on Sep. 2,  
1999, now Pat. No. 6,372,674.

(51) **Int. Cl.<sup>7</sup>** ..... **B32B 9/04**

(52) **U.S. Cl.** ..... **8/115.51; 442/153**

(58) **Field of Search** ..... **8/115.51; 442/153**

(56) **References Cited**

**U.S. PATENT DOCUMENTS**

|                |         |                      |           |
|----------------|---------|----------------------|-----------|
| 4,562,097 A    | 12/1985 | Walter et al. ....   | 427/209   |
| 5,614,591 A    | 3/1997  | Basinger et al. .... | 525/163   |
| 5,856,245 A    | 1/1999  | Caldwell et al. .... | 442/76    |
| 5,869,172 A    | 2/1999  | Caldwell ....        | 428/306.6 |
| 5,874,164 A    | 2/1999  | Caldwell ....        | 428/306.6 |
| 5,912,116 A    | 6/1999  | Caldwell ....        | 435/5     |
| 6,372,674 B1 * | 4/2002  | Lack ....            | 442/153   |

**FOREIGN PATENT DOCUMENTS**

|    |         |        |
|----|---------|--------|
| WO | 9949124 | 9/1999 |
| WO | 9949125 | 9/1999 |

\* cited by examiner

*Primary Examiner*—Yogendra N. Gupta

*Assistant Examiner*—Preeti Kumar

(74) *Attorney, Agent, or Firm*—Volpe and Koenig, P.C.

(57) **ABSTRACT**

A textile treatment process, treatment bath, and treated  
fabric are disclosed. The process imparts water repellent,  
stain resistant, and wrinkle-free properties as well as aesthe-  
tically pleasing hand properties to a fabric made in whole  
or in part of fibers having a hydroxyl group, such as  
cellulosic fibers, though immersion in an aqueous bath and  
subsequent heating for curing. The aqueous treatment bath  
contains a urea resin, polytetrafluoroethylene (PTFE) and,  
preferably, fluoroalkyl acrylate copolymer.

**20 Claims, 5 Drawing Sheets**





Figure 1

| Example A: Garment Application With Batch Processing                                  |                              |
|---------------------------------------------------------------------------------------|------------------------------|
| Pounds of Garments (fabric) Treated= 1000                                             |                              |
| Condition 1: application of 100% of bath on garment                                   |                              |
| Condition 2: application of 100% of weight of garment (weight after application=2000) |                              |
| Chemicals<br>% solids                                                                 | Actual % Solids<br>on Fabric |
| 60%                                                                                   | 0.3% Water                   |
| 22%                                                                                   | 2.2% TE-3667N (PTFE)         |
| 100%                                                                                  | 2.5% DMDHEU (22% sol.)       |
| 40%                                                                                   | 2.0% Mg Chorlide             |
| 100%                                                                                  | 0.5% NICCA NFN-158           |
|                                                                                       | Ethoxylated Alcohol          |
|                                                                                       | 0.5%                         |
|                                                                                       |                              |
|                                                                                       | Total                        |
|                                                                                       | 1000                         |
|                                                                                       | 100.0%                       |
| % of Product<br>on weight of<br>Garments/Fabric                                       |                              |
| Chemical Used                                                                         |                              |
| Garments/Fabric                                                                       |                              |
| pounds of<br>chemical on<br>Garments/Fabric                                           |                              |
| pounds of<br>chemicals needed<br>at 100% application                                  |                              |
| Chemicals<br>% of<br>bath                                                             |                              |

FIGURE 2

| Chemicals<br>% solids | Actual % Solids<br>on Fabric | Chemical Used       | % of Product<br>on weight of<br>Garments/Fabric | pounds of<br>chemical on<br>Garments/Fabric | pounds of<br>chemicals needed<br>at 50% application | Chemicals<br>% of<br>bath |
|-----------------------|------------------------------|---------------------|-------------------------------------------------|---------------------------------------------|-----------------------------------------------------|---------------------------|
|                       |                              | Water               |                                                 |                                             | 315                                                 | 63.0%                     |
| 60%                   | 0.3%                         | TE-3667N (PTFE)     | 0.5%                                            | 5                                           | 5                                                   | 1.0%                      |
| 22%                   | 2.2%                         | DMDHEU (22% sol.)   | 10.0%                                           | 100                                         | 100                                                 | 20.0%                     |
| 100%                  | 2.5%                         | Mg Chloride         | 2.5%                                            | 25                                          | 25                                                  | 5.0%                      |
| 40%                   | 2.0%                         | NICCA NFN-158       | 5.0%                                            | 50                                          | 50                                                  | 10.0%                     |
| 100%                  | 0.5%                         | Ethoxylated Alcohol | 0.5%                                            | 5                                           | 5                                                   | 1.0%                      |
|                       |                              |                     |                                                 | Total                                       | 500                                                 | 100.0%                    |

**FIGURE 3**

| Chemicals<br>Actual % Solids<br>% solids<br>on Fabric | Chemical Used            | % of Product<br>on weight of<br>Garments/Fabric | pounds of<br>chemical on<br>1000 pounds of<br>Garments/Fabric | pounds of<br>chemicals needed<br>per 500 pounds<br>of bath | Chemicals<br>% of<br>bath |
|-------------------------------------------------------|--------------------------|-------------------------------------------------|---------------------------------------------------------------|------------------------------------------------------------|---------------------------|
|                                                       | Water                    |                                                 |                                                               | 315                                                        | 63.0%                     |
| 60%                                                   | 0.3% TE-3667N (PTFE)     | 0.5%                                            | 5                                                             | 5                                                          | 1.0%                      |
| 22%                                                   | 2.2% DMDHEU (22% sol.)   | 10.0%                                           | 100                                                           | 100                                                        | 20.0%                     |
| 100%                                                  | 2.5% Mg Chorlide         | 2.5%                                            | 25                                                            | 25                                                         | 5.0%                      |
| 40%                                                   | 2.0% NICCA NFN-158       | 5.0%                                            | 50                                                            | 50                                                         | 10.0%                     |
| 100%                                                  | 0.5% Ethoxylated Alcohol | 0.5%                                            | 5                                                             | 5                                                          | 1.0%                      |
|                                                       |                          |                                                 | Total 500                                                     | 500                                                        | 100.0%                    |

FIGURE 4

**Example D: Garment Application With Continuous Processing**

Condition: application of 60% of weight of garment  
(weight of 1000 lb. of garments after bath application=1600 lb.)

| Chemicals<br>% solids | Actual %<br>on Fabric | Chemical Used       | % of Product<br>on weight of<br>Garments/Fabric | Garments/Fabric | pounds of<br>chemical on<br>1000 pounds of<br>Garments/Fabric |         | Chemicals<br>% of<br>bath |
|-----------------------|-----------------------|---------------------|-------------------------------------------------|-----------------|---------------------------------------------------------------|---------|---------------------------|
|                       |                       |                     |                                                 |                 | pounds of<br>chemicals needed<br>per 2500 pounds<br>of bath   | Total   |                           |
| 60%                   | 0.3%                  | Water               |                                                 |                 |                                                               | 1729    | 69.2%                     |
| 22%                   | 2.2%                  | TE-3667N (PTFE)     | 0.5%                                            |                 | 5                                                             | 21      | 0.8%                      |
|                       |                       | DMDHEU (22% sol.)   | 10.0%                                           |                 | 100                                                           | 417     | 16.7%                     |
| 100%                  | 2.5%                  | Mg Chorlide         | 2.5%                                            |                 | 25                                                            | 104     | 4.2%                      |
| 40%                   | 2.0%                  | NICCA NFN-158       | 5.0%                                            |                 | 50                                                            | 208     | 8.3%                      |
| 100%                  | 0.5%                  | Ethoxylated Alcohol | 0.5%                                            |                 | 5                                                             | 21      | 0.8%                      |
|                       |                       |                     |                                                 | Total           | 2500                                                          | 1000.0% |                           |

**FIGURE 5**

**BATH FOR PRODUCING WRINKLE  
FREE-WATER RESISTANT FABRICS AND  
GARMENTS**

**RELATED APPLICATION**

This application is a divisional/continuation-in-part application of U.S. patent Ser. No. 09/388,738, filed Sep. 2, 1999.

**FIELD OF THE INVENTION**

The present invention relates to the treatment of textiles, and more particularly to a treatment bath which provides a fabric having water repellent, stain resistant, and wrinkle-free properties. Most particularly, the present invention relates to a bath for producing water repellent, stain resistant, and wrinkle-free fabrics which display excellent hand and feel.

**BACKGROUND OF THE INVENTION**

U.S. Pat. No. 5,856,245 discloses an example of a barrier web comprising a fabric that has been treated with a curable shear thinned thixotropic polymer composition, the fabric being substantially impermeable to liquids, permeable to gases and impermeable to all microorganisms.

U.S. Pat. No. 5,869,172 discloses an example of processes for treating a porous substrate which involves controlled placement of modifiers through the manipulation of chemical and physical properties inherent in the modifiers to produce internally coated porous materials. The treatment involves impregnating the porous substrate with a curable thixotropic material and one or more modifying materials to impart desired properties.

U.S. Pat. Nos. 5,874,164 and 5,912,116 provide examples of a barrier web comprising a fabric that has been treated with a curable shear thinned thixotropic polymer composition. The fabric is substantially impermeable to liquids, permeable to gases and impermeable to all microorganisms. The barrier webs are either impermeable to all microorganisms or are impermeable to microorganisms of certain sizes. These patents also disclose fabrics that are capable of selectively binding certain microorganisms, particles or molecules depending upon the binding agents incorporated into the polymer before application to the fabric.

**SUMMARY OF THE INVENTION**

The present invention is directed to a textile treatment process that imparts water repellent, stain resistant, and wrinkle-free properties as well as aesthetically pleasing hand properties to a fabric made in whole or in part of fibers having a hydroxyl group, such as cellulosic fibers. The present invention is also directed to the resultant fabric of the process.

The fabrics are treated by immersion into an aqueous bath thereby applying a controlled amount of the bath to the fabric. The fabrics are then preferably dried to their natural regain, and pressed to remove unwanted wrinkles. Thereafter heat is applied to cure the reactants.

The aqueous bath is preferably formulated to apply to the fabric 8% to 14% by weight of the fabric of a reactive modified ethylene urea resin solution and 4% to 10% by weight of a crosslinking polytetrafluoroethylene additive which is at least 25% by weight polytetrafluoroethylene. Upon immersion of a fabric which has fibers having a hydroxyl group, such as cellulosic fibers, and subsequent heating, the urea resin reacts with the hydroxyl group and forms crosslinks with the polytetrafluoroethylene to impart the desired properties to the fabric.

Alternatively, the bath is formulated to apply 0.6% to 3.3% by weight of the fabric of a urea resin, preferably DMDHEU, 0.3% to 1.5% polytetrafluoroethylene (PTFE), and 1 to 4% fluoroalkyl acrylate copolymer. A bonding reaction between the urea resin and the hydroxyl group on the fabric is initiated upon immersion of the fabric and strengthened when heat is applied during the drying and curing processes.

Preferably, the bath contains a buffer to maintain pH in a range of 3.5 to 5.5 and a catalyst to speed the reaction.

Objects and advantages of the present invention will become more readily apparent to those skilled in the art upon consideration of the following detailed description which describes a preferred embodiment of the invention.

**BRIEF DESCRIPTION OF THE DRAWING(S)**

FIG. 1 is a schematic illustration of the textile treatment process according to the invention.

FIGS. 2 and 3 are tables for example baths used in batch processing.

FIGS. 4 and 5 are tables for example baths used in continuous processing.

**DETAILED DESCRIPTION OF THE  
PREFERRED EMBODIMENT(S)**

The present invention is directed to a water repellent, stain resistant, breathable, wrinkle-free fabric which retains the hand and feel of the untreated textile. The fabric is prepared by treating a textile made with preferably at least 10% fibers which have a hydroxyl group such as cellulosic fibers. The textile is immersed in a bath having a unique combination of urea resin and a fluorochemical PTFE, such as polytetrafluoroethylene (PTFE), which reacts with cellulosic fabric fibers and is cured on the fabric to form a polymer network.

The aqueous treatment bath contains a reactive modified ethylene urea resin solution such as a 22% solution of dimethylol dihydroxy ethylene urea (DMDHEU). The amount of such modified ethylene urea resin solution applied by the treatment bath preferably ranges from 8 to 14% by weight of the fabric. The amount of fluorochemical PTFE applied by the treatment bath is about 0.3% by weight and preferably ranges from 0.3% to 3% by weight. Fluoroalkyl acrylate copolymer is also preferably applied by the treatment bath at an amount ranging from 1 to 4% by weight of the fabric.

Commercial polytetrafluoroethylene additive products which are made from as low as 25% by weight powdered polytetrafluoroethylene, such as ZONYL® PTFE, which is available from E. I. du Pont de Nemours and Company can be used to provide the necessary fluorochemical copolymer PTFE and fluoroalkyl acrylate copolymer. Such additives may also be introduced in a premixed form such as ZONYL® FMX sold by Ciba Specialty Chemical Products. If ZONYL® PTFE having fluoroalkyl acrylate copolymer is used in the treatment bath, it is preferably applied by the bath at an amount ranging from 4 to 10% by weight.

The aqueous bath preferably also includes one or more additives selected from a group of buffering agents and catalysts. Buffering agents help control the acidity, or pH, of the bath and help reduce tendering of the fabric. Typical buffering agents include acetic acid, citric acid, maleic acid, and other suitable weak acids. The buffering agent is used to adjust the pH to a range of 3.5 to 5.5, preferably no more than 4.5.

A catalyst can be used to help speed the reaction so that a simple immersion technique can be used during the

treatment process instead of prolonged saturation of the fabric and to reduce curing time. Typical catalysts that can be used are parabolic catalysts such as magnesium chloride or aluminum chloride.

In one preferred formulation, a liquid premix containing fluorochemical PTFE and fluoroalkyl acrylate copolymer is used in preparing the aqueous bath. Premixed products which include a suspension agent and a surfactant, are preferred to allow the fluorochemical PTFE and fluoroalkyl acrylate copolymer to readily mix with the modified ethylene urea resin. On a weight percent basis, the treatment bath may apply 1 to 2% hexylene glycol as a suspension agent, and 0.5 to 1.5% ethoxylated aliphatic alcohol as a surfactant to the fabric being treated. If ZONYL® PTFE is used, a premixed combination of ZONYL® PTFE with hexylene glycol and ethoxylated aliphatic alcohol is ZONYL® FMX, sold by Ciba Specialty Chemicals Corporation of High Point, N.C.

In another preferred formulation, ZONYL® TE-3667N PTFE, which is an aqueous suspension of a hydrophobic colloid containing approximately 60% by total weight of 0.05 to 0.5  $\mu\text{m}$  PTFE resin particles, is used for providing at least 0.2% by weight of the fabric of PTFE via the applied bath and a 40% co-polymer solution of fluoroalkyl acrylate such as NFN-158 available from NICCA Chemical USA of Simpsonville, S.C., is used to provide at least 1% fluoroalkyl acrylate co-polymer to the fabric via the applied bath. A surfactant, such as ethoxylated aliphatic alcohol is also preferably used.

The fabrics treated in the bath are made at least in part of fibers which contain hydroxyl groups which act as a binding site for the urea resin. One type of hydroxyl containing fibers are cellulosic fibers which include natural fibers such as cotton and synthetic materials such as rayon. Accordingly, fabrics made of cotton, rayon and cotton and rayon blends are suitable for treatment using the inventive process. When the textile is immersed in the treatment bath, the DMDHEU reacts with the hydroxyl groups of fibers and acts as a binding site for the urea resin. The binding or crosslinking of the hydroxyl groups and the urea resin enhance the adhesion of the PTFE. The combination of these components results in a synergistic effect in which the fabric displays water resistant, stain resistant, and wrinkle-free properties while maintaining excellent hand.

FIG. 1 schematically illustrates the process of the present invention by which fabrics having cellulosic fibers are treated to impart water repellent, stain resistant, and wrinkle-free properties. First the aqueous treatment bath is prepared and the fabric is immersed in the bath or otherwise applied using conventional means 12. The fabric is then dried 14 to its natural regain. Where the immersion and drying steps result in wrinkling of the fabric, pressing 15 is then conducted to remove the wrinkles. Finally, the fabric is heated 16 to cure the treated fabric to impart water repellent, stain resistant, and wrinkle-free properties to the fabric.

For garments, the bath immersion may be effected in a bath process by placing the garment in a treatment vessel and immersing the garment in the aqueous bath 12. The garments are then preferably tumble dried 14 with heated air to the natural regain of the textile fibers. The natural regain of cotton is 8 to 10%, rayon 12 to 14%, and 1% for polyester so that drying time varies dependent upon whether the fabric is 100% cellulosic fiber or a blend with, for example, polyester, i.e. cotton/polyester; rayon/polyester, etc. After tumble drying, the garments are pressed to remove unwanted wrinkles 15 and directed through a heated curing

oven 16 at a temperature of 325 to 330 degrees F. preferably for at least eight to fifteen minutes to cure and crosslink the treatment composition, which imparts water resistant, stain resistant and wrinkle-free properties without destroying the natural hand or feel of the fabric.

Alternatively, garments or bolts of fabric may be treated by a conventional continuous process, where they are conveyed through the bath, wrung dry using a nip and/or air dried to natural regain, and then cured by passage through a 10 continuous processing oven. Where sheets of fabric are dried through passage through a nip, the nip may also serve to remove wrinkles thereby eliminating a separate pressing step.

After treatment, the fabric can withstand repeated washing 15 with no significant degradation of the water resistant, stain resistant and wrinkle-free properties.

In one example, a bath was prepared by mixing equal parts of a 22% aqueous solution of DMDHEU with the liquid premix described above. Acetic acid was added to 20 adjust the pH to be between 3.5 and 4.5 and magnesium chloride was added as a catalyst. The resultant aqueous bath as applied to a fabric contained by weight: about 11% DMDHEU, about 2% fluorochemical PTFE, about 2.5% fluoroalkyl acrylate copolymer, about 1.5% hexylene glycol, about 1% ethoxylated aliphatic alcohol, about 0.1% acetic acid, and about 4% magnesium chloride.

Garments made of 100% cotton fiber were immersed in the bath, dried to 8 to 10% moisture content, pressed to remove unwanted wrinkles, and cured to a temperature of 30 about 325 degrees F. for approximately 15 minutes. The resultant treated garments exhibited excellent water and stain resistant and wrinkle-free properties, even after repeated washing.

Similar results were achieved using a bath prepared by 35 mixing equal parts of a 22% aqueous solution of DMDHEU with ZONYL® FMX. Acetic acid was added to adjust the pH to be between 3 and 4.5 and magnesium chloride was added as a catalyst. The resultant aqueous bath as applied to the fabric contained by weight: about 11% DMDHEU, about 40 7% ZONYL® PTFE, about 1.5% hexylene glycol, about 1% ethoxylated aliphatic alcohol, about 0.1% acetic acid, and about 4% magnesium chloride.

Further examples are provided with reference to the tables 45 set forth in FIGS. 2-5. Examples A and B provide similar bath formulations for batch processing at two different rates of application to garments/fabric being treated. Example C and D are directed to a bath where continuous processing at two different levels of application to the garments/fabric 50 being treated. In all of the Examples A-D, the bath is a mixture of water, ZONYL® TE-3667N (60% PTFE suspension in water), a 22% by weight solution of DMDHEU, magnesium chloride, NICCA-NFN-158 solution (40% fluoroalkyl acrylate co-polymer) and ethoxylated aliphatic alcohol.

In the Examples A-D, the chemicals are mixed in the proportions indicated in the seventh column of each of the tables such that the garments absorb the percentage of the chemical indicated in the fourth column of each of the 60 tables, FIG. 2-FIG. 5. FIG. 2 provides an illustration where an equal weight of bath is applied to the garment so that after treating, and before drying, a batch of 1000 pounds of garments will weigh 2000 pounds having absorbed 1000 pounds of the bath. To produce the percentages of weight on the garment of the respective constituent bath chemicals which impart the wrinkle free and water resistant characteristics set forth in column 4 of FIG. 2, the number of 65

pounds of each material and their proportion for the bath are set forth in the sixth and seventh column of the table of FIG. 2 where 1000 pounds of bath treatment is applied to 1000 pounds of garment.

With respect to Example B, FIG. 3, 1000 pounds of garments are treated with 50% by weight of bath i.e. 500 pounds of bath. In order to provide the same percentages by weight of the desired chemicals on the garments after the bath application as in Example A, the actual pounds in proportion of chemicals for the bath at an application rate of 50% of the garment is set forth in sixth and seventh columns of FIG. 3.

As shown in FIG. 4, Example C provides a table for a bath used in continuous processing where 50% by weight of the bath is applied to the garments/fabric being treated. Since the application rate is the same for Examples B and C, the same percentage formulation for the bath is required for the continuous processing of Example C as it is for the batch processing of Example B. This is reflected in the seventh column of both examples, FIGS. 3 and 4, respectively. While Example C refers to treating 1000 pounds of garments using 500 pounds of bath at a 50% application rate, for continuous processing any weight of garments/fabric may be processed and the bath is continuously supplied as long as processing continues.

Where the bath application rate changes, the percentage of the makeup of the bath also correspondingly changes in order to maintain the same percentage of the desired chemicals being applied to the garments. For example, in Example D the rate of application of the bath is changed to 60% of the weight of the garment in comparison to Example C which is set forth for 50% application of the bath to the garments being treated. In order to have the same weight of the desired chemicals applied to the garments/fabric being treated, as reflected in the fourth column of Examples C and D, the actual bath component formulations, set forth in the seventh column, are correspondingly changed to account for the different application rates. Whether batch or continuous processing is used, one of ordinary skill of the art can easily calculate the composition of the bath to produce the desired proportionate application of chemicals on the fabric based on the application rate of the bath on the garments/fabric by simple well known mathematical calculations.

In bath processing, whether batch or continuous, the application rate is a function of a number of factors such as type of material, type of weave, fabric caliper etc. Even for an unknown fabric it is relatively easy to determine the application rate through the simple process of applying the bath to a known weight of garment and weighing the resultant garment after application of the bath to determine the total weight of the bath absorbed by the garment. In a large number of application, the application rate of the bath is about 50 or 60% by weight of the garment.

In using the combination of chemicals of Examples A-D, it is preferred that the percent of the active chemicals by weight of fabric as actually applied to the garments/fabric is in the range of 0.5 to 5% of the preferred ZONYL® TE-3667N 60% PTFE suspension and in the range of 3-15% of the preferred 22% solution of the DMDHEU. Accordingly, this results in a preferred application of 0.3 to 3% PTFE and 0.66 to 3.3% of DMHEU by weight of the fabric on the fabric. The amount of DMDHEU can be varied in accordance with the type of fabric. For example, light weight shirts of 100% cotton are preferably be treated with a bath which imparts the lower range of the DMDHEU. In

contrast, a cotton/nylon blend fabric is preferably be treated with the higher end range of DMDHEU.

Preferably, fluoroalkyl acrylate co-polymer is applied so that 1 to 4% by weight of the fabric is applied by the bath treatment. Where NICCA NFN-158 solution, which contains 40% fluoroalkyl acrylate co-polymer, is used, the bath preferably applies 2.5 to 10% NICCA NFN-158 solution to the fabric. The bath also preferably applies up to about 1% of the fabric weight of a surfactant such as ethoxylated aliphatic alcohol and up to about 4% of the fabric weight of a catalyst such as magnesium chloride. Acetic acid or the like may be used to control pH as discussed above in the range of 3.5 to 4.5.

While the invention has been described with respect to the specific formulations, other variations will be apparent to those of ordinary skill in the art and are included within the scope of the present invention.

What is claimed is:

1. An aqueous textile treatment bath for imparting water resistant, stain resistant and wrinkle-free properties to a fabric which has fibers having a hydroxyl group, such as cellulosic fibers, the aqueous bath formulated to apply to the fabric:

8% to 14% by weight of the fabric of a reactive modified ethylene urea resin solution; and

4% to 10% by weight of the fabric of a polytetrafluoroethylene additive which is at least 25% by weight of a crosslinking polytetrafluoroethylene (PTFE), whereby upon immersion of the fabric and subsequent heating, the urea resin reacts with the hydroxyl group and forms crosslinks with the polytetrafluoroethylene to impart the properties to said fabric.

2. The aqueous textile treatment bath according to claim 1 wherein said polytetrafluoroethylene additive includes a suspension of small PTFE resin particles.

3. The aqueous textile treatment bath according to claim 2 wherein said modified ethylene urea resin solution is a solution of about 22% dimethylol dihydroxy ethylene urea (DMDHEU).

4. The aqueous textile treatment bath according to claim 2 further comprising a catalyst selected from a group of parabolic acids.

5. The aqueous textile treatment bath according to claim 4 further comprising a buffering agent selected from a group of weak acids.

6. The aqueous textile treatment bath according to claim 5 wherein said modified ethylene urea resin solution is a solution of about 22% dimethylol dihydroxy ethylene urea (DMDHEU), said buffering agent is acetic acid, and said catalyst is magnesium chloride.

7. An aqueous textile treatment bath for imparting water resistant, stain resistant and wrinkle-free properties to a fabric which has fibers having a hydroxyl group, such as cellulosic fibers, the aqueous bath formulated to apply to the fabric:

0.6% to 3.3% by weight of the fabric of a reactive modified ethylene urea resin; and

at least 0.2% by weight of the fabric of a crosslinking polytetrafluoroethylene (PTFE), whereby upon immersion of the fabric and subsequent heating the urea resin reacts with the hydroxyl group and forms crosslinks with the polytetrafluoroethylene to impart the properties to said fabric.

8. The aqueous textile treatment bath according to claim 7 wherein the bath is formulated to apply 0.3% to 3% by

weight of a crosslinking polytetrafluoroethylene (PTFE) and also 1% to 4% by weight of a fluoroalkyl acrylate copolymer.

9. The aqueous textile treatment bath according to claim 8 wherein said modified ethylene urea resin is dimethylol dihydroxy ethylene urea (DMDHEU).

10. The aqueous textile treatment bath according to claim 9 further comprising a catalyst selected from a group of parabolic acids.

11. The aqueous textile treatment bath according to claim 10 wherein said catalyst comprises magnesium chloride.

12. The aqueous textile treatment bath according to claim 9 further comprising a buffering agent selected from a group of weak acids.

13. The aqueous textile treatment bath according to claim 12 wherein the buffering agent comprises acetic acid.

14. The aqueous textile treatment bath according to claim 9 further comprising a surfactant.

15. The aqueous textile treatment bath according to claim 14 wherein said surfactant comprises ethoxylated aliphatic alcohol.

16. The aqueous textile treatment bath according to claim 9 further comprising a suspension agent.

17. The aqueous textile treatment bath according to claim 16 wherein said suspension agent comprises hexylene glycol.

18. The aqueous textile treatment bath according to claim 9 where the DMDHEU is provided as a solution of about 22% DMDHEU such that 3% to 15% by weight of the fabric of that solution is applied, the PTFE is provided as a suspension of about 60% PTFE such that 0.5% to 5% by weight of the fabric of that suspension is applied, and the fluoroalkyl acrylate co-polymer is provided as a solution of about 40% fluoroalkyl acrylate co-polymer such that 2.5% to 10% by weight of the fabric of the fluoroalkyl acrylate co-polymer solution is applied.

19. The aqueous textile treatment bath according to claim 18 further comprises magnesium chloride formulated to be applied up to 4% of the fabric weight and ethoxylated aliphatic alcohol formulated to be applied up to 1% of the fabric weight.

20. The aqueous textile treatment bath according to claim 19, wherein the pH of said bath is within the range of 3.5 to 4.5.

\* \* \* \* \*

UNITED STATES PATENT AND TRADEMARK OFFICE  
**CERTIFICATE OF CORRECTION**

PATENT NO. : 6,746,491 B2  
DATED : June 8, 2004  
INVENTOR(S) : Ronnie Franklin Lack

Page 1 of 1

It is certified that error appears in the above-identified patent and that said Letters Patent is hereby corrected as shown below:

Title page,  
Item [56], **References Cited**, US PATENT DOCUMENTS, insert

|    |           |         |            |
|----|-----------|---------|------------|
| -- | 3,606,992 | 09/1971 | Aldrich    |
|    | 3,617,188 | 11/1971 | Snyder     |
|    | 3,649,165 | 03/1972 | Cotton --. |

Signed and Sealed this

Twenty-eighth Day of September, 2004



JON W. DUDAS  
*Director of the United States Patent and Trademark Office*